

# United States Patent Office

2,777,766

Patented Jan. 15, 1957

1

2,777,766

## CORROSION RESISTANT ALLOYS

William O. Binder, Niagara Falls, N. Y., assignor to Union Carbide and Carbon Corporation, a corporation of New York

No Drawing. Application June 4, 1952,  
Serial No. 291,813

4 Claims. (Cl. 75—134)

This invention relates to corrosion-resistant alloys. Media causing corrosion of metals may be classified generally as either oxidizing or reducing in chemical nature. Although many alloys exist today which are designed to resist corrosion, in general, they may not be used interchangeably for reducing and oxidizing media. Thus, the austenitic chromium-nickel steels exhibit very satisfactory resistance to attack by oxidizing agents, for example, nitric acid, but their resistance to reducing type corrosives, such as hydrochloric acid is relatively poor. On the other hand, nickel-base alloys containing substantial quantities of molybdenum have excellent resistance to reducing-type corrosives, but their resistance to oxidizing-type corrosives is not good. Furthermore, although a limited number of alloys exist which have fairly satisfactory resistance to both oxidizing and reducing corrosives, such alloys are subject to pitting in chloride solutions.

It is an object of this invention to provide alloys which have useful resistance to both oxidizing and reducing corrosive media. Another object of the invention is the provision of alloys which as well as having useful resistance to both oxidizing and reducing media, also have resistance to pitting in chloride solutions. It is also an object of the invention to provide such alloys which are hot-workable.

The invention by means of which this object is achieved comprises chromium-nickel-molybdenum-iron alloys in which the proportions of the alloying elements are balanced with respect to one another to attain the best combination of properties. The alloys of the invention contain 18% to 25% chromium; 35% to 50% nickel; 2% to 12% molybdenum; 0.1% to 5% of tantalum or columbium or both; up to 5% tungsten; up to 2.5% copper; the remainder iron and incidental impurities; the iron content being not less than 15%. As is customary with alloys of this general nature, the alloys may contain up to 1.5% manganese and up to 0.5% silicon. Carbon is of course present unavoidably, but should not exceed 0.25% and is preferably kept as low as possible, for example less than 0.1%.

Much experimental work has shown that chromium is the most effective element in the alloys of the invention for imparting resistance to oxidizing corrosives and that nickel and molybdenum are the most effective elements for imparting resistance to reducing corrosives. Since these elements tend to work against each other, that is chromium tending to lessen the effectiveness of nickel and molybdenum against reducing corrosives, and nickel and molybdenum tending to lessen the effectiveness of chromium against oxidizing corrosives, they are balanced in the alloys of the invention so that the effectiveness of each is retained insofar as possible. Since tungsten also works against chromium with regard to resistance to oxidizing corrosives, it is also taken into account when balancing the effective chromium content against the

2

nickel content. From this experimental work, the following relationship was derived:

$$5 \quad \text{Percent Cr} - \frac{2}{3}(\text{percent Mo} + 0.3(\text{percent W})) = 6.6(\text{percent Ni})^{0.25}$$

The left hand side of this equation represents "effective chromium." To attain the optimum resistance to both oxidizing and reducing media the effective chromium content of the alloys must be such that the left hand side of the equation is at least equal to the right hand side.

10 It will be observed that the above equation does not take into account the columbium or tantalum that may be present in the alloys of the invention. Within the range 0.1% to 5% these elements have no substantial detrimental effect on alloys containing chromium, nickel, molybdenum and tungsten within the ranges above defined insofar as resistance to oxidizing or reducing media is concerned.

15 On the other hand, the elements columbium and tantalum, as well as molybdenum and tungsten are, in conjunction with chromium importantly beneficial in promoting resistance to pitting in chloride solutions. Experimental work has shown that for optimum resistance to this type of corrosion the composition of the alloy should satisfy the following equation:

$$20 \quad \text{Percent Cr} + 2(\text{percent Mo}) + \frac{1}{2}(\text{percent W}) + 4(\text{percent Ta}) + 2.5(\text{percent Cb}) = 6.8(\text{percent Ni})^{0.45}$$

25 As in the case of the first equation, for the most consistently effective resistance, the alloys of the invention should be so balanced in composition that the left hand side of the equation is at least equal to the right hand side.

30 It is important that the total content of the elements molybdenum, tungsten, columbium, and tantalum, as well as chromium, be as low as possible consistent with the attainment of the desired corrosion resistance, not only because the elements are expensive but also because too high a total content of the metals of this group detrimentally affects hot-workability and increases the structural instability of the alloys. The alloys of the invention structurally are complex solid solutions which are subject to partial decomposition if exposed to temperatures between 500° C. and 900° C. The precipitate which 35 is formed by this decomposition detrimentally affects the corrosion resistance of the alloys in some environments unless special precautions are taken. Accordingly it is desirable that their composition be properly balanced in accordance with the above equation so as to minimize 40 structural instability.

45 In a properly balanced alloy the elements columbium and tantalum, in addition to improving pit resistance, minimize the loss of corrosion resistance in oxidizing media due to decomposition of the matrix solid solution during welding and stress-relieving operations. The action of 50 these elements appears to be that of retarding the decomposition rate. However, they do not render the alloy completely immune to decomposition, and if optimum corrosion resistance is required after welding, the alloys should be annealed by heating to 1100° C. to 1150° C. followed by cooling relatively rapidly.

55 To provide good resistance to oxidizing media after welding and stress-relieving, about 1% of columbium or tantalum is required when the molybdenum content is about 3%. If the molybdenum content is higher, say 6%, it is preferred to add 2% of these elements to the alloy. Tantalum and columbium may be present together, and although they may be present in any ratio, a 1:1 ratio 60 is preferred for economic reasons.

65 For optimum resistance to pitting after welding and stress-relieving, the nickel content of the alloys should be

restricted to the range 40% to 50%. Nickel stabilizes the solid-solution matrix and reduces the rate at which the solid solution decomposes below 900° C. It increases susceptibility to pitting, however, which must be

Typical of the results obtained in such tests are those set forth in the following table. The corrosion rates in the acids are expressed in terms of inches penetration per month in the table.

| Alloy No. | Percent Composition; Remainder Fe and 1.5% Max. Mn and 0.5% Max. Si |    |    |   |      |      |      |      | Results of Corrosion Tests |                            |                                         |                                                    |
|-----------|---------------------------------------------------------------------|----|----|---|------|------|------|------|----------------------------|----------------------------|-----------------------------------------|----------------------------------------------------|
|           | Cr                                                                  | Ni | Mo | W | Cb   | Ta   | Cu   | C    | Boiling 65% Nitric Acid    | Boiling 10% Sulphuric Acid | Aerated 10% Hydrochloric Acid at 70° C. | 5% FeCl <sub>3</sub> -10% NaCl at 25° C., 72 Hours |
| 1.        | 20                                                                  | 35 | 6  | — | 0.8  | 1    | —    | low  | 0.0015                     | 0.00299                    | 0.0390                                  | No pitting.                                        |
| 2.        | 22                                                                  | 35 | 6  | — | —    | 1    | —    | 0.05 | 0.00104                    | Not tested                 | Not tested                              | Do.                                                |
| 3.        | 22                                                                  | 35 | 7  | — | —    | —    | 1.61 | 0.05 | 0.00160                    | 0.00400                    | 0.0350                                  | Do.                                                |
| 4.        | 22                                                                  | 45 | 6  | — | 2.32 | —    | —    | 0.07 | 0.00110                    | 0.00230                    | 0.0220                                  | Do.                                                |
| 5.        | 22                                                                  | 45 | 6  | — | 1.43 | 0.58 | —    | 0.05 | 0.00095                    | Not tested                 | Not tested                              | Very slight pitting.                               |
| 6.        | 22                                                                  | 45 | 6  | — | 0.98 | 1.2  | —    | 0.06 | 0.00103                    | do                         | do                                      | Do.                                                |
| 7.        | 22                                                                  | 45 | 6  | — | 0.75 | 1.71 | —    | 0.06 | 0.00097                    | do                         | do                                      | Do.                                                |
| 8.        | 22                                                                  | 45 | 6  | — | 0.97 | 0.97 | —    | 0.05 | 0.00091                    | do                         | do                                      | Do.                                                |
| 9.        | 22                                                                  | 45 | 6  | — | 1.12 | —    | —    | 0.06 | 0.00220                    | 0.00160                    | do                                      | Do.                                                |
| 10.       | 25                                                                  | 40 | 6  | — | 1    | 1    | 0.25 | 0.04 | 0.00087                    | Not tested                 | 0.0204*                                 | Do.                                                |
| 11.       | 22                                                                  | 45 | 6  | — | 1    | 1    | 0.98 | 0.04 | 0.00148                    | do                         | 0.0210*                                 | Do.                                                |
| 12.       | 22                                                                  | 45 | 6  | — | 1    | 1    | 2    | 0.04 | 0.00142                    | 0.00119                    | 0.0176*                                 | Do.                                                |
| 13.       | 22                                                                  | 45 | 6  | — | 1    | —    | —    | —    | —                          | —                          | —                                       | —                                                  |

\*Results obtained in one 48-hour period.

overcome by increasing the chromium and molybdenum contents. Since the latter elements promote the decomposition of the solid solution, it is important not to increase the amount of these elements beyond that required to overcome the influence of nickel.

Copper may be present in the alloys of the invention in minor proportions as an impurity. It may be added as an alloying constituent, and relatively small proportions of copper are beneficial in increasing the resistance to corrosion of the alloys in reducing acids such as dilute hydrochloric acid and sulfuric acid in concentrations of about 10% to 50%. Resistance to attack by hot phosphoric acid is also enhanced by the presence of copper. Although copper is beneficial in quantities up to 2.5%, larger quantities tend to lower the resistance of the alloys to pitting and contact corrosion. Therefore the alloys generally should contain not more than 2.5% copper, and a preferred range is 0.25% to 1%. In these small proportions copper may be omitted from consideration in the equations above set forth despite indications that in the alloys of this invention copper behaves like nickel and somewhat more powerfully.

Many hundreds of tests of the alloys of the invention have been made, and such tests have demonstrated that the alloys possess useful resistance to oxidizing corrosives, reducing corrosives and solutions of the type which cause pitting. For such tests samples 1 inch wide, 1½ inches long and ¼ inch thick were machined from ¼ inch plate which had been rolled directly (at initial rolling temperature of 1150° C. to 1200° C.) from ingots 2 inches square. The samples were heated 30 minutes at 1100° C.; cooled in air, descaled in a 20% nitric acid-2% hydrofluoric acid bath at 70° C., drilled for mounting, and polished. Before immersion in the testing solutions, each sample was degreased and carefully measured and weighed.

Different samples prepared as described were immersed in four different media; boiling 65% nitric acid; boiling 10% sulfuric acid; aerated 10% hydrochloric acid at 70° C. and 5% ferric chloride-10% sodium chloride at 25° C. The samples were suspended in the acids for three 48 hour periods being removed and weighed between periods, and results of three such 48 hour periods were averaged. In the chloride solution the samples were placed on the bottom of the glass jar holding the solution to simulate a concentration cell and to obtain an indication of the resistance of the sample to contact corrosion. The samples were kept in the chloride solution for 72 consecutive hours.

It will be seen from the above table that the alloys of the invention possess useful resistance to oxidizing media, reducing media, and to chloride solutions.

That the alloys of the invention are hot-workable is demonstrated by hot-twist tests. In such tests a hot-rolled sample consisting of a round bar about 22 inches long by ¾ inch in diameter and having a reduced section about 8 inches long and ⅝ inch diameter in the center, is twisted to failure. The reduced section is heated uniformly for a distance of about 3½ inches on each side of the center, and the bar is twisted at a constant speed of 180 revolutions per minute. The total number of twists and the initial torque are observed. In the following table typical test results are compared with typical results obtained on conventional stainless steels. Alloy "A" in the table is an alloy according to this invention containing 22% chromium; 45% nickel; 6% molybdenum; 1% columbium; 1% tantalum; 1.5% manganese; 0.5% silicon; remainder iron. Alloy "B" is a steel containing 19% chromium; 9% nickel; 1.3% manganese; 0.4% silicon; 0.08% carbon; remainder iron and Alloy "C" is a steel containing 18% chromium; 15% nickel; 3% molybdenum; 1.5% manganese; 0.5% silicon; 0.05% carbon; remainder iron.

| Alloy | Test Temp., °C. | Torque, in.-lb. | No. of Twists Before Fracture |
|-------|-----------------|-----------------|-------------------------------|
| A     | 1,150           | 920             | 32                            |
| A     | 1,200           | 770             | 31                            |
| B     | 1,150           | 360             | 35                            |
| B     | 1,200           | 320             | 42                            |
| C     | 1,150           | 560             | 29                            |
| C     | 1,200           | 490             | 32                            |

The data in the above table show the high order of hot-workability which can be obtained from a well balanced alloy in accordance with this invention.

In general, the maximum hot-working temperature range for the alloys is 1150° to 1175° C. For optimum hot-workability, the extreme limits of the broad composition range should be avoided as the alloys decrease in hot-workability as the chromium and molybdenum contents increase. The addition of tantalum benefits the hot-workability of the alloys, and it is more helpful than columbium.

The alloys of the invention may be welded by conventional methods.

A specific alloy according to the invention which has

particularly good resistance to oxidizing media, reducing media, and chloride solutions contains about 22% chromium; 45% nickel; 6% molybdenum; 1% columbium; 1% tantalum; 1.5% manganese; 0.5% silicon; 0.05% carbon; the remainder iron.

This is a continuation-in-part of my application Serial No. 100,769, filed June 22, 1949, now abandoned.

What is claimed is:

1. An alloy article resistant to oxidizing-type and reducing-type corrosive media, which article is composed of an alloy consisting of 18% to 25% chromium; 35% to 50% nickel; 2% to 12% molybdenum; 0.1% to 5% in the aggregate of at least one metal selected from the group consisting of tantalum and columbium; up to 5% tungsten; up to 2.5% copper; less than 0.25% carbon; the remainder iron and incidental impurities, the iron content being at least 15% and the individual constituents of said alloy being so proportioned that the left hand side of the following equation is at least equal to the right hand side:

$$\text{Percent Cr} - \frac{2}{3}(\text{percent Mo} + 0.3) \quad (15) \\ (\text{percent W}) = 6.6(\text{percent Ni})^{0.25}$$

2. An alloy article resistant to pitting-type corrosive media, which article is composed of an alloy consisting of 18% to 25% chromium; 40% to 50% nickel; 2% to 12% molybdenum; 0.1% to 5% in the aggregate of at least one metal selected from the group consisting of tantalum and columbium; up to 5% tungsten; up to 1% copper; less than 0.25% carbon; the remainder iron and 30 incidental impurities, the iron content being at least 15% and the individual constituents of said alloy being so proportioned that the left hand side of the following equation is at least equal to the right hand side:

$$\text{Percent Cr} + 2(\text{percent Mo}) + \frac{1}{2}(\text{percent W}) + \quad (35) \\ 4(\text{percent Ta}) + 2.5(\text{percent Cb}) = 6.8(\text{percent Ni})^{0.45}$$

3. An alloy article resistant to corrosive media of the oxidizing type, the reducing type and the pitting type, which article is composed of an alloy consisting of 18% 40

to 25% chromium; 35% to 50% nickel; 2% to 12% molybdenum; 0.1% to 5% in the aggregate of at least one metal selected from the group consisting of tantalum and columbium; up to 5% tungsten; up to 2.5% copper less than 0.25% carbon; the remainder iron and incidental impurities, the iron content being at least 15% and the individual constituents of said alloy being so proportioned that the left hand sides of both of the following equations are at least equal to the respective right hand sides thereof:

$$\text{Percent Cr} - \frac{2}{3}(\text{percent Mo} + 0.3) \quad (15) \\ (\text{percent W}) = 6.6(\text{percent Ni})^{0.25}$$

$$\text{Percent Cr} + 2(\text{percent Mo}) + \frac{1}{2}(\text{percent W}) + \quad (20) \\ 4(\text{percent Ta}) + 2.5(\text{percent Cb}) = 6.8(\text{percent Ni})^{0.45}$$

4. An alloy article resistant to corrosive media of the oxidizing type, the reducing type and the pitting type, which article is composed of an alloy having substantially the following composition: 22% chromium; 45% nickel; 6% molybdenum; 1% columbium; 1% tantalum; 1.5% maximum manganese; 0.5% maximum silicon; less than 0.1% carbon; the remainder iron and incidental impurities.

#### References Cited in the file of this patent

##### UNITED STATES PATENTS

|           |                  |       |               |
|-----------|------------------|-------|---------------|
| 2,162,253 | Grossman         | ----- | June 13, 1939 |
| 2,245,366 | Rohn et al.      | ----- | June 10, 1941 |
| 2,373,490 | Mohling          | ----- | Apr. 10, 1945 |
| 2,403,128 | Scott et al.     | ----- | July 2, 1946  |
| 2,423,738 | Thielemann       | ----- | July 8, 1947  |
| 2,432,617 | Franks et al.    | ----- | Dec. 16, 1947 |
| 2,451,547 | German           | ----- | Oct 19, 1948  |
| 2,504,453 | Rotherham et al. | ----- | Apr. 18, 1950 |
| 2,553,330 | Post et al.      | ----- | May 15, 1951  |

##### OTHER REFERENCES

Iron Age, vol. 161, March 18, 1948, pages 73-75.